



US008852753B2

(12) **United States Patent**  
**Matsumura et al.**

(10) **Patent No.:** **US 8,852,753 B2**  
(45) **Date of Patent:** **Oct. 7, 2014**

(54) **GALVANIZED STEEL SHEET**

(75) Inventors: **Kenichiro Matsumura**, Tokyo (JP);  
**Makoto Nakazawa**, Tokyo (JP);  
**Masahiro Yui**, Tokyo (JP); **Takehiro**  
**Takahashi**, Tokyo (JP)

(73) Assignee: **Nippon Steel & Sumitomo Metal Corporation**, Tokyo (JP)

(\*) Notice: Subject to any disclaimer, the term of this patent is extended or adjusted under 35 U.S.C. 154(b) by 0 days.

(21) Appl. No.: **13/521,302**

(22) PCT Filed: **Jul. 9, 2010**

(86) PCT No.: **PCT/JP2010/061703**

§ 371 (c)(1),  
(2), (4) Date: **Jul. 10, 2012**

(87) PCT Pub. No.: **WO2012/004889**

PCT Pub. Date: **Jan. 12, 2012**

(65) **Prior Publication Data**

US 2012/0288734 A1 Nov. 15, 2012

(51) **Int. Cl.**

**B32B 15/04** (2006.01)  
**B32B 15/18** (2006.01)  
**C23C 28/00** (2006.01)  
**C23C 2/28** (2006.01)  
**C23C 2/06** (2006.01)  
**C23C 2/02** (2006.01)

(52) **U.S. Cl.**

CPC ..... **C23C 2/06** (2013.01); **C23C 28/321** (2013.01); **C23C 28/345** (2013.01); **C23C 2/28** (2013.01); **C23C 2/02** (2013.01)

USPC ..... **428/659**; 428/633; 428/336; 428/340

(58) **Field of Classification Search**

USPC ..... 428/659, 632, 633, 630, 631, 639, 658,

428/684, 685, 687, 212, 213, 215, 216, 219,  
428/220, 332, 335, 336, 340, 704, 341, 469,  
428/472, 472.1, 472.2, 472.3

See application file for complete search history.

(56)

**References Cited**

## U.S. PATENT DOCUMENTS

|               |        |                              |
|---------------|--------|------------------------------|
| 5,409,553 A   | 4/1995 | Sagiyama et al.              |
| 5,518,769 A   | 5/1996 | Sagiyama et al.              |
| 5,525,431 A * | 6/1996 | Kanamaru et al. .... 428/623 |

## FOREIGN PATENT DOCUMENTS

|    |           |        |
|----|-----------|--------|
| EP | 0 473 154 | 3/1992 |
| EP | 1 002 886 | 5/2000 |

(Continued)

## OTHER PUBLICATIONS

Machine Translation, Unno et al., JP 08-092714, Apr. 1996.\*

(Continued)

Primary Examiner — Michael E La Villa

(74) Attorney, Agent, or Firm — Kenyon & Kenyon LLP

(57) **ABSTRACT**

The present invention provides a galvanized steel sheet including: a steel sheet; and a galvanizing layer provided on a surface of the steel sheet; wherein the galvanizing layer includes an amorphous coating layer having an inorganic oxoacid salt and metallic oxide on a surface layer of the galvanizing layer; the galvanizing layer includes a  $\zeta$  phase and a  $\delta_1$  phase; the galvanizing layer includes, by mass, 8 to 13% of Fe; Zn in the metallic oxide exists up to an outermost surface layer of the amorphous layer; and an X-ray diffraction intensity ratio I, which is obtained by dividing an X-ray diffraction intensity of the  $\zeta$  phase at  $d=0.126$ , after removing background intensity, by an X-ray diffraction intensity of the  $\delta_1$  phase at  $d=0.126$ , after removing background intensity, is 0.06 to 0.35.

**9 Claims, 7 Drawing Sheets**



---

| (56)                     | References Cited |         | JP                                                                                                                                                                                                               | 2007-217784 | 8/2007  |
|--------------------------|------------------|---------|------------------------------------------------------------------------------------------------------------------------------------------------------------------------------------------------------------------|-------------|---------|
| FOREIGN PATENT DOCUMENTS |                  |         | TW                                                                                                                                                                                                               | 200940722   | 10/2009 |
|                          |                  |         | TW                                                                                                                                                                                                               | 200949012   | 12/2009 |
| OTHER PUBLICATIONS       |                  |         |                                                                                                                                                                                                                  |             |         |
| EP                       | 1 233 265        | 8/2002  | International Search Report dated Aug. 25, 2009, issued in corresponding PCT Application No. PCT/JP2009/062599.                                                                                                  |             |         |
| EP                       | 2 495 346        | 9/2012  | International Search Report dated Aug. 17, 2010, issued in corresponding PCT Application No. PCT/JP2010/061703.                                                                                                  |             |         |
| EP                       | 2 495 347        | 9/2012  | Taiwanese Notice of Allowance, dated Feb. 20, 2013, issued in corresponding Taiwanese application No. 099122493, with an English translation of the Search Report only.                                          |             |         |
| JP                       | 64-068456        | 3/1989  | Canadian Office Action, dated May 16, 2013, issued in corresponding Canadian application No. 2786639.                                                                                                            |             |         |
| JP                       | 03-191045        | 8/1991  | Jiang et al., "Effect of galvannealing process on powder residence and microstructure of galvannealing coatings of ultra-low carbon steel sheets," Gangtic Yanjiu Xucba (2012), 22(3) pp. 33-38 (Abstract only). |             |         |
| JP                       | 04-000360        | 1/1992  | Extended European Search Report dated Dec. 5, 2013 issued in corresponding EP Application No. 10854443.8.                                                                                                        |             |         |
| JP                       | 04-006258        | 1/1992  |                                                                                                                                                                                                                  |             |         |
| JP                       | 04-013855        | 1/1992  |                                                                                                                                                                                                                  |             |         |
| JP                       | 4088196          | 3/1992  |                                                                                                                                                                                                                  |             |         |
| JP                       | 04-176878        | 6/1992  |                                                                                                                                                                                                                  |             |         |
| JP                       | 08-092714        | 4/1996  |                                                                                                                                                                                                                  |             |         |
| JP                       | 2819427          | 10/1998 |                                                                                                                                                                                                                  |             |         |
| JP                       | 2002-012958      | 1/2002  |                                                                                                                                                                                                                  |             |         |
| JP                       | 2003-138361      | 5/2003  |                                                                                                                                                                                                                  |             |         |
| JP                       | 2003-171751      | 6/2003  |                                                                                                                                                                                                                  |             |         |
| JP                       | 2004-190074      | 7/2004  |                                                                                                                                                                                                                  |             |         |
| JP                       | 2006-183090      | 7/2006  |                                                                                                                                                                                                                  |             |         |

\* cited by examiner

FIG. 1



FIG. 2A



FIG. 2B



**FIG. 3**



FIG. 4



FIG. 5



FIG. 6



FIG. 7



FIG. 8



## 1

## GALVANIZED STEEL SHEET

This application is a national stage application of International Application No. PCT/JP2010/061703, filed Jul. 9, 2010.

## TECHNICAL FIELD OF THE INVENTION

The present invention relates to a galvanized steel sheet.

## BACKGROUND ART

Galvanized and galvannealed steel sheets (GA), which are excellent in continuous spot welding and corrosion resistance after painting, are used in a large amount as steel sheets for automobiles. Galvanized and galvannealed steel sheets initially had problems of "powdering" which is an phenomenon that a stiff galvanizing layer is crushed in powder form and exfoliated during press forming in a case that the galvanizing layer is too much alloyed (that is, in a case that the  $\Gamma$  phase that includes body-centered cubic crystal of Zn and Fe intermetallic compound ( $Fe_3Zn_{10}$ ) with 20-28 mass % of Fe is plenty) to make the galvanizing layer stiff. Further, as for a damage of the galvanizing layer, there were problems of "flaking" which is a phenomenon that a galvanizing layer is flaked and exfoliated during press forming under the high surface pressure, in a case that the galvanizing layer is insufficiently alloyed (that is, in a case that the  $\zeta$  phase that includes monoclinic crystal of Zn and Fe intermetallic compound ( $FeZn_{10}$ ) with 5.5-6.2 mass % of Fe is plenty) to induce an adhesion between the galvanizing layer and the die or the punch. However, due to advanced galvanizing layer controlling technology and pressing technology, galvanized and galvannealed steel sheets are being used without significant problems. In order to increase the powdering resistance,  $\Gamma$  phase generation in an interface between a galvanizing layer and steel substrate is usually reduced in amount. Meanwhile, in order to increase the flaking resistance,  $\zeta$  phase in a galvanizing surface layer is usually reduced in amount.

Patent Document 1 discloses a galvanized and galvannealed steel sheet having 1.0  $\mu m$  or less of  $\Gamma$  phase in an interface between a galvanizing layer and a steel substrate, the galvanizing layer having a galvanizing surface layer which does not include a  $\eta$  phase, which is a hexagonal Zn phase including not more than 0.003 mass % of Fe, or the above-mentioned  $\zeta$  phase.

Patent Document 2 discloses a galvanized and galvannealed steel sheet having  $\Gamma$  phase in a thickness of not more than 0.5  $\mu m$ , and having a galvanizing layer which does not include  $\eta$  phase or  $\zeta$  phase at the galvanizing surface layer.

Patent Document 3 discloses a galvanized and galvannealed steel sheet having a galvanizing layer on a surface of the steel sheet and having a surface roughness  $R_{max}$  of not greater than 8  $\mu m$ .

Patent Document 4 discloses a galvanized and galvannealed steel sheet wherein the surface coverage of the  $\zeta$  phase and the X-ray diffraction intensity ratio between the  $\zeta$  phase and other phases are determined to be in specific ranges.

Another approach to improve press formability is a series of techniques by providing a lubricating coat on a surface of the galvanized steel sheet instead of controlling the galvanizing layer as described above.

Patent Document 5 discloses a galvanized steel sheet including coats I and II on a galvanizing surface layer, wherein the coat I has an adhesion-preventing function and has one or more metal oxides/hydroxides selected from Mn,

## 2

Mo, Co, Ni, Ca, Cr, V, W, Ti, Al and Zn as a major component, and wherein the coat II has a rolling-lubricating function and has one or two kinds of oxygen acids selected from P and B as a major component. The coat II gradually increases in concentration toward an interface with galvanizing layer, and the coat II gradually increases in concentration toward a surface of the sheet.

Patent Document 6 discloses a galvanized and galvannealed steel sheet having a flat portion on a surface of an iron-zinc alloy galvanizing layer, the flat portion being provided with an oxide layer which includes: a Zn-based oxide as a major component; a thickness of not less than 8 nm and not more than 200 nm; and an interface width of not less than 25 nm and not more than 500 nm.

Patent Document 7 discloses a galvanized steel sheet which includes a crystalline phosphated coat formed on a surface.

## RELATED ART DOCUMENT

## Patent Document

[Patent Document 1] Japanese Unexamined Patent Application, First Publication No. H01-068456

[Patent Document 2] Japanese Unexamined Patent Application, First Publication No. H04-013855

[Patent Document 3] Japanese Unexamined Patent Application, First Publication No. H03-191045

[Patent Document 4] Japanese Unexamined Patent Application, First Publication No. H08-092714

[Patent Document 5] Japanese Unexamined Patent Application, First Publication No. H04-176878

[Patent Document 6] Japanese Unexamined Patent Application, First Publication No. 2003-171751

[Patent Document 7] Japanese Unexamined Patent Application, First Publication No. 2007-217784

## DISCLOSURE OF THE INVENTION

## Problem to be Solved by the Invention

However, in the galvanized and galvannealed steel sheets disclosed in Patent Document 1 and Patent Document 2, neither  $\eta$  phase nor  $\zeta$  phase exists in the galvanizing surface layer and the thickness of  $\Gamma$  phase is small. These galvanizing layers are therefore formed by a substantially single  $\delta_1$  phase that includes a hexagonal crystal of Zn and Fe intermetallic compound ( $FeZn_7$ ) with 7-11.4 mass % of Fe. Although these disclosed steel sheets have an ideal structure of galvanizing layer to control both powdering resistance and flaking resistance, slidability during press forming is lower than those of the steel sheets disclosed in Patent Document 5, Patent Document 6, and Patent Document 7 which include a lubricating coat provided on a surface of a galvanized steel sheet.

The galvanized and galvannealed steel sheet disclosed in Patent Document 3 includes  $\zeta$  phase existing near the galvanizing surface layer and has a certain roughness imparted to the galvanizing surface layer in order to compensate for reduced flaking resistance. The effect, however, is limited.

The galvanized and galvannealed steel sheet disclosed in Patent Document 4 also includes  $\zeta$  phase in order to improve chemical conversion treatability and cathodic electrodeposition coatability. In terms of both the powdering resistance and the flaking resistance, however, the galvanized and galvannealed steel sheet disclosed in Patent Document 4 has no ideal structure of galvanizing layer structure. The galvanized and galvannealed steel sheet disclosed in Patent Document 4

is inferior to those disclosed in Patent Document 5, Patent Document 6, and Patent Document 7 in slidability during press forming.

Meanwhile, as to the galvanized and galvannealed steel sheet disclosed in Patent Document 5, the galvannealed steel sheet to which a lubricating coat is provided on the surface layer of the galvanized steel sheet can achieve preferable slidability during press forming irrespective of whether the  $\zeta$  phase exists in the galvanizing surface. As a result, the occurrence of fracture is suppressed even if a large wrinkle suppressing force (blank holding force, BHF) is applied at the time of press forming. However, at the same time, a large wrinkle suppressing force is required to eliminate the occurrence of wrinkles. That is, even if the lower limit of the BHF with which fractures occur increases, the lower limit of the wrinkle suppressing force which is required for eliminating the wrinkle increases. Therefore, the BHF range in which neither wrinkles nor fractures occur, that is, the range for achieving press forming still remains the same as those of the related art.

The galvanized and galvannealed steel sheets disclosed in Patent Document 6 and Patent Document 7 can achieve preferable slidability during press forming irrespective of whether the  $\zeta$  phase exists in the galvanizing surface layer. The effect, however, is smaller than that of the steel sheet disclosed in Patent Document 5. The range for achieving press forming still remains the same as those of the related art.

As described above, the related arts are excellent in both of powdering resistance and flaking resistance, or slidability during press forming, but fail to extend the employable BHF range (wrinkle suppressing force), that is, the range for achieving press forming. It is therefore desirable to further improve press formability, that is, to extend the BHF (wrinkle suppressing force) range that is the range for achieving press forming in which neither wrinkles nor fractures occur.

#### Means for Solving the Problem

For solving the foregoing problems, the present invention employs the following.

(1) A first aspect of the present invention is a galvanized steel sheet including: a steel sheet; and a galvanizing layer in an amount of not less than 20 g/m<sup>2</sup> and not more than 100 g/m<sup>2</sup>, the galvanizing layer being provided on a surface of the steel sheet and containing Zn as a main component; wherein the galvanizing layer includes an amorphous coating layer having an inorganic oxoacid salt and metallic oxide on a surface layer of the galvanizing layer; the galvanizing layer includes a  $\zeta$  phase and a  $\delta_1$  phase; the galvanizing layer includes, by mass, 8 to 13% of Fe; Zn in the metallic oxide exists up to an outermost surface layer of the amorphous layer; and an X-ray diffraction intensity ratio I, which is obtained by dividing an X-ray diffraction intensity of the  $\zeta$  phase at d=0.126, after removing background intensity, by an X-ray diffraction intensity of the  $\delta_1$  phase at d=0.126, after removing background intensity, is 0.06 to 0.35.

(2) In the galvanized steel sheet according to (1), the galvanizing layer may include a  $\Gamma$  phase having an average thickness of 1.5 gm or less.

(3) In the galvanized steel sheet according to (1), the galvanizing layer may include Al in an amount of not less than 0.10 g/m<sup>2</sup> and not more than 0.25 g/m<sup>2</sup>.

(4) In the galvanized steel sheet according to (1), the galvanizing layer may include Ni in an amount of more than 0 g/m<sup>2</sup> and not more than 0.40 g/m<sup>2</sup>.

(5) In the galvanized steel sheet according to (4), the galvanizing layer includes Al in an amount of not less than 0.15 g/m<sup>2</sup> and not more than 0.45 g/m<sup>2</sup>.

(6) In the galvanized steel sheet according to any one of (1) to (5), the inorganic oxoacid salt may include at least one of P and B.

(7) In the galvanized steel sheet according to any one of (1) to (5), the metallic oxide may include at least one of metallic oxides of Mn and Al.

(8) In the galvanized steel sheet according to any one of (1) to (5), a total amount of P and B in the inorganic oxoacid salt may be not less than 1 mg/m<sup>2</sup> and not more than 250 mg/m<sup>2</sup>; and a total amount of Mn, Mo, Co, Ni, Ca, V, W, W, Ti and Ce in the metallic oxide including Zn may be not less than 1 mg/m<sup>2</sup> and not more than 250 mg/m<sup>2</sup>.

(9) In the galvanized steel sheet according to any one of (1) to (5), Zn existing in the outermost layer of the amorphous coating layer is provided so that a chemical compound of a phosphorus-containing oxoacid and a zinc becomes a major component.

#### Effects of the Invention

According to the configuration described in (1), a component with an adhesion-preventing function, an inorganic oxoacid salt with a rolling-lubricating function, and a metallic oxide exist in a uniformly mixed manner in an amorphous coating layer. Further, as to the structure of the galvanizing layer, a predetermined amount of the  $\zeta$  phase is made to exist in the surface layer. A synergistic effect generated by the lubricating coat and the structure of the galvanizing layer can provide a hot-dipped galvanized steel sheet that is excellent in lubricity and chemical conversion treatability. The steel sheet also has an extended range for achieving press forming as compared with those of the related art. Then, a higher yield can be obtained in the press forming of the steel sheets for automobile bodies more efficiently than in the related art. In addition, the possibility of the die and punch design can be expanded to produce variously designed press formed articles. Therefore, the commercial value of automobiles can be increased.

According to the configuration described in (2), a galvanized steel sheet having preferable powdering resistance can be provided.

According to the configuration described in (3), since the structure of galvanizing layer according to (1) can be obtained easily, a galvanized steel sheet having an extended range for achieving press forming can be provided.

According to the configurations described in (4) and (5), since generation of the  $\zeta$  phase in the galvanizing layer can further be controlled, a galvanized steel sheet having further extended range for achieving press forming can be provided.

According to the configurations described in (6), (7), and (8), since the structure of galvanizing layer according to (1) can be obtained easily, a galvanized steel sheet having a further extended range for achieving press forming can be provided.

According to the configuration described in (9), since appropriate lubricity is obtained, a galvanized steel sheet having a further extended range for achieving press forming can be provided.

#### BRIEF DESCRIPTION OF THE DRAWINGS

FIG. 1 is a graph illustrating removal of background intensity during obtaining an I value on the basis of a result of X-ray diffraction analysis of a galvanized steel sheet using an

## 5

equation of the X-ray diffraction intensity ratio I of  $\zeta$  phase and  $\delta_1$  phase in a galvanizing layer.

FIG. 2A is a graph illustrating the results of depth analysis by AUGER electron spectroscopy of a lubricating coat of a galvanized steel sheet according to a first embodiment of the present invention.

FIG. 2B is a graph illustrating the results of depth analysis by AUGER electron spectroscopy of a lubricating coat of a galvanized steel sheet according to a second embodiment of the present invention.

FIG. 3 is an SEM image in which the area where the lubricating coat is analyzed to the depth direction is represented by a white lined box.

FIG. 4 is spectra of 3s level Zn and 2p level P during a state analysis of a coat surface in the depth direction by X-ray photoelectron spectroscopy.

FIG. 5 is a spectrum of 2p level Zn during a state analysis of the coat surface in the depth direction by X-ray photoelectron spectroscopy.

FIG. 6 is a schematic diagram illustrating a structure of the galvanized steel sheet.

FIG. 7 shows examples of the present invention and comparative examples in Table 3, with the horizontal axis that represents X-ray diffraction intensity ratio I of the  $\zeta$  phase and the  $\delta_1$  phase regarding the ratio of the  $\zeta$  phase and the  $\delta_1$  phase in the galvanizing layer, and the vertical axis that represents the value obtained by dividing the lower limit wrinkle suppressing force ( $\beta$ ) with which fractures occur by the lower limit wrinkle suppressing force ( $\alpha$ ) which is required for eliminating wrinkles.

FIG. 8 shows examples of the present invention and comparative examples in Table 4, with the horizontal axis that represents X-ray diffraction intensity ratio I of the  $\zeta$  phase and the  $\delta_1$  phase regarding the ratio of the  $\zeta$  phase and the  $\delta_1$  phase in the galvanizing layer, and the vertical axis that represents the value obtained by dividing the lower limit wrinkle suppressing force ( $\beta$ ) with which fractures occur by the lower limit wrinkle suppressing force ( $\alpha$ ) which is required for eliminating wrinkles.

## EMBODIMENT OF THE INVENTION

The present inventors have studied a technique to provide a lubricating coat on a surface of a galvanized steel sheet as described in Patent Document 5 in order to solve the related art problems. In the related art, it was considered, as suitable conditions to provide an extended compression range for achieving press forming, that the steel sheet has a coat with an adhesion-preventing function which gradually increases concentration toward an interface with a galvanizing layer, and a coat with a rolling-lubricating function which gradually increases concentration toward a surface of the coating layer, i.e., toward an outer surface of the galvanizing layer. If the related art concept is applied to a galvanized and galvannealed steel sheet, the steel sheet has greater slidability although the galvanizing layer structure is disadvantageous to slidability. Therefore, it has been considered that the galvanizing layer structure has no influence on the slidability. The inventors have studied, instead of sticking to these two of related art concepts, about an ideal structure of galvanizing layer structure and an ideal structure of coat to provide an extended range of a wrinkle suppressing force, that is, an extended range for achieving press forming in which neither wrinkles nor fractures occur. As a result, it has been found that the range of the applicable wrinkle suppressing force, that is, the range for achieving press forming can be extended by a synergistic effect of a lubricating coat and a galvanizing layer

## 6

structure, wherein the lubricating coat has a component with an adhesion-preventing function and a component with a rolling-lubricating function which are mixed together, and wherein the galvanizing layer structure includes a predetermined amount of the  $\zeta$  phase in the surface layer.

The suitable structure of coat structure of the related art exhibits great lubricity even when low surface pressure is applied, because of a galvanizing surface including a highly concentrated rolling-lubricating component and because of a sliding interface provided between the rolling-lubricating component and the adhesion-preventing component. The related art therefore has a deficiency that wrinkles are likely to occur. This deficiency is eliminated by distributing both the rolling-lubricating component and the adhesion-preventing component in the lubricant coat. However, as described in Patent Document 5, with such a countermeasure only, there is a problem that the limit surface pressure for occurrence of galling becomes low when worked under high surface pressure, which may be disadvantageous to the occurrence of fractures during press forming. Then, the inventors studied to impart an equivalent adhesion-preventing function by making a coat stiffer than that of the related art. As a result, it was discovered that the limit surface pressure for the occurrence of galling is improved and the lower limit force ( $\beta$ ) with which a fracture occurs during press forming is increased by making a certain amount of the  $\zeta$  phase having relatively high reactivity exist in the galvanizing surface layer and taking a larger amount of Zn in the lubricating coat using a Zn dissolution reaction from the galvanizing surface layer so that Zn exists even in the outermost layer of the coating layer. From this knowledge, the inventors found that together with lowering the below-mentioned lower limit wrinkle suppressing force ( $\alpha$ ) which is required for eliminating wrinkles, the initial object of extending the compression range for achieving press forming can be achieved. It was also found that Zn in the coating outermost layer which includes a chemical compound of phosphorus-containing oxoacid and zinc as a major component may provide further suitable lubricity. It is important to appropriately control the amount of the remaining  $\zeta$  phase, since an excessively large amount of the remaining  $\zeta$  phase may impair the slidability and may cause fractures.

The inventors further studied and found that, in order to make a certain amount of the  $\zeta$  phase exist in the galvanizing surface layer, it is preferred to employ a heating pattern of "rapidly heating at a high temperature and then cooling by natural cooling or gas-water cooling" in a galvannealing (alloying) process. The inventors also found that, in order to have the component with the adhesion-preventing function, the component with the rolling-lubricating function and Zn exist in mixed state in the coating layer and to have Zn exist in the outermost layer of the coating layer, a coat is preferably formed with a treating solution containing an inorganic oxoacid salt and a metallic oxide. The inventors further found that it was advantageous to form the coat by roll coating while appropriately controlling the concentration in the treating solution and the sheet temperature immediately just before the process.

Hereinafter, embodiments of the present invention will be described in detail.

First, components of a galvanized steel sheet according to first embodiment of the present invention will be described in detail. The galvanizing layer according to the present embodiment includes Zn as a major component, and Fe in a content of not less than 8% and not more than 13% by mass.

Here, "includes Zn as a major component" means a state in which Zn is included in the amount of not less than 50% by mass.

If the Fe content in the galvanizing layer is less than 8% by mass, because of insufficient alloy forming, corrosion resistance after painting becomes poor and the excessively large amount of the  $\zeta$  phase may impair slidability to generate flaking during press forming. On the other hand, if the Fe content exceeds 13% by mass, the  $\Gamma$  phase becomes thick to impair powdering resistance. In order to provide higher flaking resistance, powdering resistance and corrosion resistance after painting, the Fe content is preferably kept not less than 8.5% by mass and not more than 12.5, more preferably, not less than 9% by mass and not more than 12% by mass.

If the steel sheet is used for automobiles, the amount of the galvanizing layer is preferably not less than 20 g/m<sup>2</sup> and not more than 100 g/m<sup>2</sup>, for one surface. If the amount of the galvanizing layer is less than 20 g/m<sup>2</sup>, corrosion resistance becomes insufficient, and 30 g/m<sup>2</sup> or more is more preferable. If the amount of the galvanizing layer exceeds 100 g/m<sup>2</sup>, continuous spot weldability becomes low, and 70 g/m<sup>2</sup> or less is more preferable.

In order to keep satisfactory powdering resistance, the thickness of the  $\Gamma$  phase is preferably not more than 1.5  $\mu\text{m}$ , more preferably not more than 1  $\mu\text{m}$ , and further preferably 0.8  $\mu\text{m}$ .

If the amount of the galvanizing layer is not less than 20 g/m<sup>2</sup> and not more than 100 g/m<sup>2</sup>, the total Al concentration in the galvanizing bath should be in a range of not less than 0.11% by mass and not more than 0.15% by mass for properly alloying the coating layer. If the total Al concentration in the galvanizing bath is lower than 0.11% by mass, the alloying process becomes out of control and leads to overall alloy. If the total Al concentration in the galvanizing bath is higher than 0.15% by mass, delayed alloying may cause deterioration in manufacturing efficiency. With the above conditions, the total Al amount in the galvanizing layer, i.e., the total Al amount derived from the conditions of the barrier layer and the galvanizing bath of the initial alloying, falls within a range of not less than 0.10 g/m<sup>2</sup> and not more than 0.25 g/m<sup>2</sup>. The amount of Al in the galvanizing layer is preferably controlled to be not less than 0.13 g/m<sup>2</sup> and not more than 0.22 g/m<sup>2</sup>, and more preferably, not less than 0.15 g/m<sup>2</sup> and not more than 0.20 g/m<sup>2</sup>.

Regarding the ratio of the  $\zeta$  phase and the  $\delta_1$  phase in the galvanizing layer, the X-ray diffraction intensity ratio I of these  $\zeta$  phase and  $\delta_1$  phase is set to be in a range of not less than 0.06 and not more than 0.35, when the X-ray diffraction intensity ratio I is represented by the following Equation (1).

$$I = \zeta(d=0.126 \text{ nm})/\delta_1(d=0.127 \text{ nm}) \quad (1)$$

In Equation (1),  $\zeta(d=0.126 \text{ nm})$  represents the value of the X-ray diffraction intensity of the  $\zeta$  phase when the interplanar spacing distance (d) is 0.126 nm. Further,  $\delta_1(d=0.127 \text{ nm})$  represents the value of the X-ray diffraction intensity of  $\delta_1$  phase when the interplanar spacing distance (d) is 0.127 nm.

Since the  $\zeta$  phase contains a large amount of zinc when compared with that of the  $\delta_1$  phase, small value of the X-ray diffraction intensity ratio I means that the amount of zinc in the galvanizing layer is small, and as a result, the adhesion to a die or a punch can be reduced and the slidability improves. If the X-ray diffraction intensity ratio I is lower than 0.06, slidability is excessively high and the lower limit wrinkle suppressing force ( $\alpha$ ) required for eliminating wrinkles increases, and at the same time, the amount of Zn taken into the amorphous coating layer including an inorganic oxoacid salt and a metallic oxide by dissolving from the galvanizing

surface layer decreases, thus, the limit of the wrinkle suppressing force with which a fracture occurs decreases, thereby narrowing the range for achieving press forming. If the X-ray diffraction intensity ratio I is higher than 0.35, the slidability is insufficient and the lower limit wrinkle suppressing force ( $\alpha$ ) which is required for eliminating wrinkles decreases, but at the same time, the lower limit wrinkle holding force ( $\beta$ ) with which a fracture is generated also decreases, thus, the range for achieving press forming is also narrowed in this case. It is preferable for the X-ray diffraction intensity ratio to be in a range of not less than 0.10 and not more than 0.35, and more preferably, in a range of not less than 0.15 and not more than 0.30.

The X-ray diffraction intensity of  $\zeta$  (d=0.126 nm) and the X-ray diffraction intensity of  $\delta_1$  (d=0.127 nm) are the values after removal of the background intensity. A process of removing the background intensity will be illustrated in FIG. 1. In FIG. 1, the horizontal axis represents the incidence angle of the X-ray and the vertical axis represents diffraction intensity.

In FIG. 1, K1 is a line that represents the background intensity having a peak 19 corresponding to the  $\delta_1$  phase and K2 is a line that represents the background intensity having a peak 20 corresponding to the  $\zeta$  phase. Further, L is a line that represents intensity of  $\delta_1$  (d=0.127 nm) after removal of the background intensity in the  $\delta_1$  phase and M is a line that represents intensity of  $\zeta$  (d=0.126 nm) after removal of the background intensity in the  $\zeta$  phase.

Next, components of a galvanized steel sheet according to the second embodiment of the present invention will be described in detail. The galvanizing layer according to the present embodiment includes Zn as a major component, Fe in a content of not less than 8% and not more than 13% by mass, Al in an amount of not less than 0.15 g/m<sup>2</sup> and not more than 0.45 g/m<sup>2</sup>, and Ni in an amount of more than 0 g/m<sup>2</sup> and not more than 0.40 g/m<sup>2</sup>.

In the second embodiment, the steel sheet is pre-plated with a small amount of Ni and then immersed in a hot-dip galvanizing bath with an Al concentration higher than that in the first embodiment to galvanize the same. The steel sheet is thus galvanized in order to further control the generation of the phase. According to a Zn—Al—Fe ternary alloy phase diagram, the phase is not likely to generate and the 6 phase is likely to generate in a galvanizing solution of higher Al concentration. If the Al concentration in the galvanizing bath is simply increased, many Fe—Al barrier layers may generate in an interface with the steel substrate and thus the alloying process is delayed, thereby lowering manufacturing efficiency. In order to prevent this phenomenon, the steel sheet is pre-plated with a small amount of Ni and then immersed in a galvanizing bath in which the pre-plated Ni and Al in the bath are made to react with each other near an interface with the steel sheet. In this manner, Al concentration near the interface is lowered and the amount of the Fe—Al barrier layer generated at the interface is controlled so as not to be excessively large. Since Al concentration in the deposit galvanizing layer is high, the phase is not likely to generate during alloying.

The amount of Ni in the galvanizing layer is determined to be more than 0 g/m<sup>2</sup> and not more than 0.40 g/m<sup>2</sup> on the basis of an appropriate range of the amount of Ni to be pre-plated. A suitable amount of Ni for pre-plating is not less than 0.10 g/m<sup>2</sup> and not more than 0.50 g/m<sup>2</sup>. When the pre-plated steel sheet is immersed in a hot-dip galvanizing bath, the pre-plating is partly dissolved in the galvanizing bath and removed. Thus, as the amount of Ni remaining in the galvanizing layer, more than 0 g/m<sup>2</sup>, or more preferably, more than 0.07 g/m<sup>2</sup>, and not more than 0.40 g/m<sup>2</sup> is determined. It

should be noted that if the amount of pre-plating Ni is more than 0.10 g/m<sup>2</sup>, generation of unplated portions can be eliminated. Meanwhile, if the amount of the pre-plating Ni exceeds 0.50 g/m<sup>2</sup>, the reaction of Ni and Al in the bath becomes unfortunately excessively rapid and as a result, an uneven barrier layer is formed to impair the appearance of the produced alloy.

The amount of Al in the galvanizing layer is determined to be not less than 0.15 g/m<sup>2</sup> and not more than 0.45 g/m<sup>2</sup> on the basis of an appropriate range of Al concentration in the galvanizing bath. If the amount of the pre-plating Ni is not less than 0.10 g/m<sup>2</sup> and not more than 0.50 g/m<sup>2</sup>, the total Al concentration in the galvanizing bath should be in a range of not less than 0.16% by mass and not more than 0.20% by mass. If the Al concentration in the galvanizing bath is less than 0.16% by mass, the alloying process becomes out of control and leads to overalloy. If the Al concentration in the galvanizing bath is more than 0.20% by mass, delayed alloying may cause deterioration in manufacturing efficiency. If the amount of the galvanizing layer is not less than 20 g/m<sup>2</sup> and not more than 100 g/m<sup>2</sup>, the total Al amount in the galvanizing layer, i.e., the total Al amount derived from the barrier layer and the galvanizing bath of the initial alloying is in a range of not less than 0.15 g/m<sup>2</sup> and not more than 0.45 g/m<sup>2</sup>.

In the second embodiment, when compared with the first embodiment, the total Al concentration in the galvanizing bath can be increased as described above, and since the  $\zeta$  phase is hard to be generated and  $\delta_1$  phase is likely to be generated, the value of the X-ray diffraction intensity ratio I can be controlled to be lower.

Next, components of the lubricating coat will be described in detail. In both the first and second embodiments, the lubricating coat formed on the surface of the galvanizing layer is an amorphous coating layer of an inorganic oxoacid salt and a metallic oxide.

Examples of a suitable inorganic oxoacid salt that can be used for forming the coat in the first and second embodiments include oxygen acid containing P and a salt thereof. Examples of other materials include boric acid, which is oxygen acid containing P, and a salt thereof. These may be used alone or in mixture thereof. The mixture preferably includes the oxygen acid containing P. Further, the mixture may include oxide colloids of Si, Al, Ti and the like. It is considered that these materials achieve lubricating function, basically due to rolling particles crushed at the time of press forming.

Meanwhile, the metallic oxide may be an oxide or hydroxide of Zn, Al, Ni, Mn, Mo, Co, Ni, Ca, V, W, Ti, Ce, and the like. Among these components added to a reaction solution, Zn, Al and Ni are taken into the lubricating coat when Zn, Al and Ni are dissolved from the galvanizing layer to the reaction solution. Zn is an especially important component to reinforce the function to prevent the galvanizing layer from being adhered to the die and punch. These components taken into the lubricating coat are detectable in depth directional atom analysis by AUGER electron spectroscopy. Existence of Zn in the coat outermost layer can be detected, without sputtering, through detection of Zn by elemental analysis on a sample surface by AUGER electron spectroscopy and X-ray photoelectric spectroscopy.

The amount of each component of the inorganic oxoacid salt as the total contents of P and B, and the metallic oxide as the total contents of Zn, Al, Ni, Mo, Co, Ni, Va, V, W, Ti and Ce is suitably not less than 1 mg/m<sup>2</sup> and not more than 250 mg/m<sup>2</sup>. If the amount of each component is less than 1 mg/m<sup>2</sup>, effects of the component are insufficient. If the amount of each component is more than 250 mg/m<sup>2</sup>, an adverse effect is

made to the chemical conversion treatability. A more preferred amount of each component is not less than 3 mg/m<sup>2</sup> and not more than 150 mg/m<sup>2</sup>.

The lubricating coat significantly differs from the related art in that the inorganic oxoacid salt and the metallic oxide which includes Zn exist in the lubricating coat and that Zn oxides are provided even in the outermost layer of the coating layer.

In the suitable technique disclosed in Patent Document 5, a P-containing component with a rolling-lubricating function has increased concentration toward a surface of the coating layer, and a Mn-containing component with an adhesion-preventing function has strong concentration at the interface with steel substrate in the coating layer. The results of the glow discharge spectroscopy analysis are illustrated in a drawing.

For comparison with the related art, the results of the depth analysis by AUGER electron spectroscopic analysis corresponding to the first and the second embodiments are illustrated in FIGS. 2A and 2B. The analysis results relating to the technique disclosed in Patent Document 5 and the analysis results according to the first and the second embodiments will be compared. First, in the technique disclosed in the related art patent Document 5, the P-containing component and the Mn-containing component have peaks at explicitly different positions. The Zn exists only in the inner layer of the lubricating coat. On the other hand, the present invention includes Zn in the lubricating coat in a significantly higher amount than that of the related art and includes Zn existing even in the outermost layer of the lubricating coat.

That is, the galvanized steel sheet according to the present embodiment differs from the related art in that the Zn component exist even in the outermost layer of the lubricating coat. With this configuration of the coat, the range for achieving press forming can be expanded.

Here, Zn in the lubricating coat may be generated so that the chemical compound of phosphorus-containing oxoacid and Zn become major components (50% or more). In other words, Zn in the outermost layer may be majorly (50% or more) generated so as to be presented in a state of a chemical compound of phosphorus-containing oxoacid and zinc (salt). The state of Zn in the coat is identified by X-ray photoelectron spectroscopy. Spectroscopic analysis was conducted by, using an X-ray photoelectron spectrometer PHI5600 available from Ulvac-Phi Inc., sputtering the coat surface at 2 nm (in terms of SiO<sub>2</sub>) a minute in an analyzing area of having a diameter 0.8 mm at an Ar pressure of 10<sup>-2</sup> Pa and accelerating voltage of 4 kV. The results of the spectroscopic analysis with an electrostatic hemisphere analyzer using an Alka X-ray as the X-ray source while varying the sputtering time are illustrated in FIGS. 4 and 5. FIG. 4 illustrates 2p spectra P and 3s spectra Zn in a region from the outermost layer to a depth of 18 nm. The horizontal axis represents the binding energy (eV). It is understood that the major component is a chemical compound of phosphorus-containing oxoacid and zinc in a region from the outermost layer to a depth of 2 nm, is a mixture of substantially the same amount of zinc phosphate, a chemical compound of phosphorus-containing oxoacid and zinc, and a zinc oxide and zinc metal are substantially the same amount at the depth of 4 nm, and the major component is a zinc oxide and zinc metal in a region from a depth of 6 nm to 18 nm. FIG. 5 illustrates a 2p spectrum of Zn of the same sample. The horizontal axis represents binding energy (eV). Similarly, it is understood that the major component is a chemical compound of phosphorus-containing oxoacid and zinc in a region from the outermost layer to a depth of 2 nm, a chemical compound of phosphorus-containing oxoacid and

## 11

zinc, a zinc oxide and a zinc metal are substantially the same amount at the depth of 4 nm, and the major component is a zinc oxide and zinc metal in a region from a depth of 6 nm to 18 nm.

Next, manufacturing conditions of the galvanized steel sheet according to the embodiments of the present invention will be described. Conditions regarding the galvanizing layer will be described first.

In this embodiment, a predetermined amount of the phase is made to exist in the galvanizing layer. The thickness of the  $\Gamma$  phase is determined to be not more than 1.5  $\mu\text{m}$  and preferably not more than 1  $\mu\text{m}$ , and further preferably not more than 0.8  $\mu\text{m}$ .

The first aspect is to employ a heating pattern of "rapidly heating at a high temperature using an electric induction heater or the like and then natural cooling, gas-water cooling, or the like" during an alloying process with the total Al concentration in the galvanizing bath being not less than 0.11% by mass and not more than 0.15% by mass. It is effective that the top temperature for alloying is higher than the peritectic temperature of the  $\zeta$  phase and becomes lower than the peritectic temperature during natural cooling. Although the peritectic temperature of the  $\zeta$  phase is 530°C. in the Zn—Fe binary alloy phase diagram, the  $\zeta$  phase is not likely to generate as a primary crystal in an Al-containing bath at a temperature of not less than 500°C.

It is preferred from the viewpoint of growth suppression of the  $\Gamma$  phase to shorten the retention time after heating, and to cool promptly. In particular, the alloying temperature is not lower than 470°C. to not higher than 600°C. and more preferably not lower than 500°C. to not higher than 530°C. The retention time is not longer than 25 seconds, more preferably not longer than 5 seconds. The cooling speed during natural cooling is not higher than 25°C./sec, more preferably not lower than 4°C./sec to not higher than 8°C./sec. The galvanizing layer is preferably cooled to about 350°C.

As second aspect, the steel sheet may be pre-plated with Ni in an amount of not less than 0.10 g/m<sup>2</sup> and not more than 0.50 g/m<sup>2</sup>, and then, a heating pattern of "rapidly heating at a high temperature using an electric induction heater or the like and then natural cooling, gas-water cooling or the like" may be employed during an alloying process with the total Al concentration in the galvanizing bath being not less than 0.16% by mass and not more than 0.20% by mass. Since the Al concentration in the bath is high, it is preferred that the alloying temperature is determined to be as high as not lower than 510°C. to not higher than 560°C., the retention time is determined to be not longer than 3 seconds, the cooling speed during the natural cooling is determined to be not less than 2°C./sec and not more than 4°C./sec and cooled to about 450°C., and then mist-cooled. According to the second aspect, as compared with the first aspect, even if the  $\Gamma$  phase is equivalent in thickness, the  $\zeta$  phase can be reduced in amount. Therefore, an extended range for achieving press forming where neither wrinkles nor fractures occur can be provided.

In either aspect, it is important to employ a heating pattern of rapidly heating at a high temperature and then natural cooling, gas-water cooling or the like. An undesirable heating pattern in which the sheet is heated at a low temperature and kept at such temperature for a while may produce sheets with an undesirable ratio of the  $\Gamma$  phase and the  $\zeta$  phase, for example, the  $\Gamma$  phase becomes excessively thick with no remaining  $\zeta$  phase, or the  $\Gamma$  phase is thin with an excessively large amount of the  $\zeta$  phase.

Next, manufacturing conditions of the lubricating coat of the galvanized steel sheet according to the embodiments of the invention will be described. The lubricating coat accord-

## 12

ing to the embodiments of the invention includes the inorganic oxoacid salt and the metallic oxide in a mixed state. Such a coat configuration is established by roll-coating using a treating solution which includes components of an inorganic oxoacid salt and a metallic oxide while controlling concentration and the sheet temperature of the galvanized steel sheet to a suitable range. A reverse roll-coating may alternatively be employed.

As preferred examples of the component which generates 10 the inorganic oxoacid salt, P-containing oxygen acid (phosphoric acid, phosphorous acid, hypophosphorous acid or the like), boric acid or the like, and the salts thereof may be used. An oxide colloid of Si, Al, Ti or other elements may be added. As preferred examples of the component which generates the 15 metallic oxide, for example, regarding Mn, an inorganic salt of manganese sulfate, manganese nitrate or permanganate may be used. In addition, oxide or hydroxide of Zn, Al, Ni, Mo, Co, Ni, Ca, V, W, Ti or Ce may be added, and for generating such oxide or hydroxide, metal nitrate salt, carbonate salt, ammonium salt or sulfuric acid salt may be used. 20 In addition, if necessary, sulfuric acid, nitric acid or the like may be added for increasing a stability of the treating solution.

The total concentration of the treating solution is not less 25 than 5 g/l and not more than 30 g/l. The total concentration herein is the sum of the concentration of P, B, Zn, Mn and the like not including oxygen. If the total concentration is less than 5 g/l, production efficiency of the lubricating coat becomes poor which reduces the threading speed. If the total 30 concentration exceeds 30 g/l, excessively uneven distribution is likely to be made in the lubricating coat. The temperature of the treating solution is preferably not less than 10°C. and not more than 50°C. The sheet temperature of the galvanized steel sheet immediately before the coat is formed is not less than 30°C. and not more than 70°C. Such a temperature range is advantageous in dissolving Zn when the sheet is made to contact with the treating solution and in forming a 35 coat and drying the formed coat. If the temperature is below 30°C., fewer effects will be exhibited. If the temperature exceeds 70°C., the amount of dissolved Zn will become 40 excessively large, which weakens the lubricating coat.

In order to make a chemical compound of phosphorus-containing oxoacid and zinc be the major component of Zn in the coat outermost layer, it is desired to increase the concentration 45 of oxygen acid containing P in the treating solution, lower the drying temperature of the coat as low as possible, and shorten the drying time. Preferably, the concentration of oxygen acid containing P is not less than 10 g/l and the coat is dried at a temperature of not more than 60°C. for not longer than 5 seconds. If the above conditions are not applied, zinc 50 oxide to be generated increases in amount.

The steel sheets that can be used in the embodiments of the invention are not to be limited, however, if high press formability is required for the steel sheet, an extremely low carbon 55 steel sheet that is excellent in deep drawability and expandability is particularly preferred. For example, a steel sheet in which Ti or Nb is added to eliminate solute C is properly used, and if necessary, a steel sheet containing P, Mn, Si, B or other elements to reinforce the same can be used. Such steel sheets can achieve the effects of the present invention without any problem. Further, a steel sheet may inevitably include tramp elements, such as Cr, Cu, Ni, and Sn.

The steel sheets according to the embodiments of the present invention can achieve synergistic effects of a lubricating coat structure which includes components with the adhesion-preventing function and components with the rolling-lubricating function in mixed state and a galvanizing

## 13

layer structure in which a predetermined amount of the  $\zeta$  phase is made to exist in the surface. Therefore, when compared with the related art steel sheets, an employable range of wrinkle suppressing force, that is, a range for achieving press forming can be extended. As a result, steel sheets in which the value obtained by dividing the lower limit wrinkle suppressing force ( $\beta$ ) with which fractures occur by the lower limit wrinkle suppressing force ( $\alpha$ ) which is required for eliminating wrinkles is preferably more than 1.21, more preferably more than 1.25, more preferably more than 1.27, and further preferably more than 1.30 can be obtained.

## Example 1

Next, the invention will be described with reference to examples. The invention, however, is not limited to these examples.

## (1) Test Specimens

The composition of sample steel sheets are shown in Table 1. Cold-rolled steel sheets with 0.7 mm thickness were used.

## (2) Galvanizing Conditions

The test specimen was degreased, heated to 800°C. in a 4% H<sub>2</sub>-N2 atmosphere and left for 60 s. Then, the test specimen was air-cooled to 470°C., immersed in a hot-dip galvanizing bath of 460°C. for 3 s and wiped to control the amount. The obtained test specimen was heated and alloyed under the conditions shown in Table 2, which will be described later, air-cooled to 350°C., mist-cooled and then taken out.

## (3) Analysis of Galvanizing Layer

The amounts of Zn, Fe, and Al in the galvanizing layer were measured by inductively coupled plasma (ICP atomic emission spectrometry) after the galvanizing layer was dissolved with inhibitor-containing hydrochloric acid to which 0.6% of hexamethylenetetramine manufactured by WAKO Corporation Limited was added. These amounts were summed to obtain the total amount. The value of the above-mentioned Equation relating to the X-ray diffraction intensity ratio I of the  $\zeta$  phase and the  $\delta_1$  phase regarding the ratio of the  $\zeta$  phase and the  $\delta_1$  phase in the galvanizing layer was calculated after the background intensity was removed by the method illustrated in FIG. 1 from the result obtained by the X diffraction. The thickness of the  $\Gamma$  layer was obtained by etching a cross section of the galvanizing layer with, for example, nital (an etching solution consisting of alcohol and nitric acid) and observing the neighborhood of the interface with steel substrate by an optical microscope. For each sample N=3, ten sufficiently spaced normal visual fields were observed and thicknesses thereof were measured to provide an average thickness of the  $\Gamma$  phase.

## (4) Conditions for Forming Coat

The treating solutions having a composition shown in Table 2 were used. The galvanized steel sheet was pre-heated to a predetermined temperature and then treated in either of the following manners:

RC: roll coating and then drying (sheet temperature: 50°C.);

Dip: immersing, rinsing and drying (sheet temperature: 50°C.); and

EC: electrolytic treatment, rinsing and drying (sheet temperature: 50°C.).

## (5) Analysis of Coat

After the coat was dissolved in a chromic acid solution, the amount of each element was determined by inductively coupled plasma (ICP atomic emission spectrometry). The amount of the inorganic oxoacid salt shown in Table 3 is the sum of the amounts of P and B, and the amount of the metallic oxide shown in Table 3 is the sum of the amounts of Mn, Zn, Al, Ce and Ti.

## 14

The coat structure was subject to depth analysis regarding a region to a depth of 10 nm from the surface layer in a selected area of about 3  $\mu\text{m} \times 3 \mu\text{m}$  in a flat portion without significant pits and lands of the galvanizing surface layer as illustrated in FIG. 3. At the same time, elemental analysis for each sputtering event (of every 0.1 min) was conducted by AUGER electron spectroscopy at the sputter speed of about 10 nm/min. The state in which P, Mn and Zn are included in a uniform mixture without intentional unevenness as illustrated in FIGS. 2A and 2B and Zn exists even in the coating layer surface is herein referred to as type A. The state in which, as illustrated in Fifth drawing of Patent Document 5, the P-containing component has a peak at the surface layer side and the Mn-containing component has a peak at the inner layer side, which peaks are explicitly different in position, and no Zn exists in the coating layer surface is herein referred to as type B.

Regarding Zn in the coat outermost layer, the spectra illustrated in FIGS. 4 and 5 were obtained by X-ray photoelectron spectroscopy and then examined whether or not Zn exists even in the coat outermost layer and whether Zn in the outermost layer is mainly a chemical compound of phosphorus-containing oxoacid and zinc (P—Zn) or zinc oxide based (ZnO).

## (6) Friction Coefficient

The sample with the coat formed thereon was cut into pieces of 17 mm in width and 300 mm in length. NOX RUST®550HN (Available from Parker Industries Inc.) was applied to each piece in an amount of 1 g/m<sup>2</sup>. Then a draw bead test was conducted at a drawing speed of 500 mm/min. The drawing force was measured while varying the pressure force from 200 kgf-800 kgf (i.e., from  $1.96 \times 10^3 \text{ N}$ - $7.84 \times 10^3 \text{ N}$ ). An inclination is obtained with the pressure force plotted to the horizontal axis and the obtained value was multiplied by  $\frac{1}{2}$  to provide the friction coefficient.

## (7) Wrinkle Generating Limit and Fracture Generating Limit

The sample with the coat formed thereon was punched to a diameter of 90 mm and then subject to a cylinder-shape forming test with a punch diameter of 50 mm (4R) and a dice diameter of 54 mm (4R). The lower limit force ( $\alpha$ ) with which wrinkles eliminate and the lower limit force ( $\beta$ ) with which fractures occur were obtained while varying the wrinkle suppressing force (blank holder force) from 3 tons to 7 tons (i.e., from  $2.94 \times 10^4 \text{ N}$  to  $6.93 \times 10^4 \text{ N}$ ).

## (8) Chemical Conversion Treatability

The sample with the coat formed thereon was degreased and surface-controlled as prescribed using a commercially-available chemical conversion treatment solution (SD5000 available from Nippon Paint Co., Ltd.). Subsequently, the sample was subject to a chemical conversion treatment. The sample was observed by SEM, determined to be "good" if it has a uniform coat and determined to be "fair" if it has an uncoated portion in a section of an area rate not more than 10%.

## (9) Comparative Material

Comparative materials having no coating thereon (32 and 33 in Table 3) and a comparative material having, instead of the coating, 3 g/m<sup>2</sup> of Fe—Zn electroplating (Fe: 80%) (34 in Table 3) were prepared.

TABLE 1

| Steel | C     | Si    | Mn   | P     | S     |
|-------|-------|-------|------|-------|-------|
| I     | 0.001 | 0.011 | 0.11 | 0.005 | 0.004 |
| II    | 0.002 | 0.005 | 0.64 | 0.025 | 0.007 |

TABLE 2

| Treating solution | Inorganic oxide | Metallic oxide      |
|-------------------|-----------------|---------------------|
| ①                 | Phosphoric acid | Manganese nitrate   |
| ②                 | Phosphoric acid | Permanganate        |
| ③                 | Phosphoric acid | Manganese sulfate   |
| ④                 | Boric acid      | Sulfate cerium (IV) |
|                   | Nitric acid     | Manganese nitrate   |
|                   | Phosphoric acid | Nickel nitrate      |

The performance evaluation results are shown in Table 3. In Table 3, articles 1 to 24 relate to galvanized steel sheets

according to an embodiment of the invention and articles 25 to 34 relate to galvanized steel sheets according to comparative examples. FIG. 7 shows examples of the present invention and comparative examples in Table 3, with the horizontal axis that represents X-ray diffraction intensity ratio I of the  $\zeta$  phase and the  $\delta_1$  phase regarding the ratio of the  $\zeta$  phase and the  $\delta_1$  phase in the galvanizing layer, and the vertical axis that represents the value obtained by dividing the lower limit wrinkle suppressing force ( $\beta$ ) with which fractures occur by the lower limit wrinkle suppressing force ( $\alpha$ ) which is required for eliminating wrinkles.

TABLE 3

| Article | Steel | Treating solution | Configuration of surface treatment |        |                        |       |                                     |      | Coating layer                       |                |                                     |
|---------|-------|-------------------|------------------------------------|--------|------------------------|-------|-------------------------------------|------|-------------------------------------|----------------|-------------------------------------|
|         |       |                   | Galvanizing layer                  |        |                        | Type  | Applied amount (mg/m <sup>2</sup> ) | Type | Applied amount (mg/m <sup>2</sup> ) | Type           | Applied amount (mg/m <sup>2</sup> ) |
|         |       |                   | Applied amount (g/m <sup>2</sup> ) | Fe (%) | Al (g/m <sup>2</sup> ) |       |                                     |      |                                     |                |                                     |
| 1       | I     | ①                 | 20                                 | 10.2   | 0.13                   | 0.215 | 0.75                                | P    | 15                                  | Mn, Zn, Al     | 7                                   |
| 2       | I     | ①                 | 30                                 | 10.1   | 0.14                   | 0.237 | 0.70                                | P    | 20                                  | Mn, Zn, Al     | 10                                  |
| 3       | I     | ①                 | 45                                 | 10.8   | 0.16                   | 0.327 | 0.70                                | P    | 25                                  | Mn, Zn, Al     | 15                                  |
| 4       | I     | ①                 | 60                                 | 9.7    | 0.18                   | 0.288 | 0.70                                | P    | 50                                  | Mn, Zn, Al     | 35                                  |
| 5       | II    | ①                 | 70                                 | 11.7   | 0.19                   | 0.070 | 1.20                                | P    | 15                                  | Mn, Zn, Al     | 5                                   |
| 6       | II    | ①                 | 70                                 | 9.4    | 0.20                   | 0.230 | 0.65                                | P    | 75                                  | Mn, Zn, Al     | 50                                  |
| 7       | I     | ②                 | 25                                 | 9.2    | 0.17                   | 0.323 | 0.60                                | P    | 15                                  | Mn, Zn, Al     | 7                                   |
| 8       | I     | ②                 | 30                                 | 9.5    | 0.17                   | 0.236 | 0.65                                | P    | 25                                  | Mn, Zn, Al     | 15                                  |
| 9       | I     | ②                 | 45                                 | 9.7    | 0.17                   | 0.331 | 0.65                                | P    | 40                                  | Mn, Zn, Al     | 20                                  |
| 10      | I     | ②                 | 50                                 | 9.3    | 0.17                   | 0.342 | 0.65                                | P    | 40                                  | Mn, Zn, Al     | 30                                  |
| 11      | I     | ②                 | 50                                 | 10.0   | 0.17                   | 0.187 | 0.80                                | P    | 50                                  | Mn, Zn, Al     | 30                                  |
| 12      | II    | ②                 | 60                                 | 9.7    | 0.17                   | 0.189 | 0.75                                | P    | 50                                  | Mn, Zn, Al     | 50                                  |
| 13      | II    | ②                 | 70                                 | 9.2    | 0.17                   | 0.275 | 0.72                                | P    | 150                                 | Mn, Zn, Al     | 100                                 |
| 14      | I     | ③                 | 70                                 | 8.8    | 0.22                   | 0.158 | 0.45                                | P, B | 20                                  | Mn, Zn, Al, Ce | 20                                  |
| 15      | I     | ③                 | 30                                 | 10.9   | 0.19                   | 0.302 | 0.90                                | P, B | 35                                  | Mn, Zn, Al, Ce | 20                                  |
| 16      | I     | ③                 | 45                                 | 9.5    | 0.17                   | 0.315 | 0.60                                | P, B | 35                                  | Mn, Zn, Al, Ce | 20                                  |
| 17      | I     | ③                 | 50                                 | 10.1   | 0.18                   | 0.332 | 0.85                                | P, B | 50                                  | Mn, Zn, Al, Ce | 25                                  |
| 18      | I     | ③                 | 50                                 | 9.7    | 0.17                   | 0.314 | 0.70                                | P, B | 50                                  | Mn, Zn, Al, Ce | 30                                  |
| 19      | II    | ③                 | 60                                 | 9.3    | 0.17                   | 0.304 | 0.65                                | P, B | 70                                  | Mn, Zn, Al, Ce | 50                                  |
| 20      | II    | ③                 | 70                                 | 8.5    | 0.17                   | 0.206 | 0.45                                | P, B | 200                                 | Mn, Zn, Al, Ce | 150                                 |
| 21      | I     | ④                 | 30                                 | 9.5    | 0.18                   | 0.341 | 0.55                                | P    | 15                                  | Mn, Zn, Al, Ni | 10                                  |
| 22      | I     | ④                 | 50                                 | 9.5    | 0.17                   | 0.298 | 0.60                                | P    | 20                                  | Mn, Zn, Al, Ni | 20                                  |
| 23      | II    | ④                 | 50                                 | 9.6    | 0.16                   | 0.313 | 0.65                                | P    | 30                                  | Mn, Zn, Al, Ni | 20                                  |
| 24      | II    | ④                 | 50                                 | 9.5    | 0.17                   | 0.307 | 0.60                                | P    | 40                                  | Mn, Zn, Al, Ni | 25                                  |
| 25      | I     | ①                 | 50                                 | 8.5    | 0.17                   | 0.464 | 0.55                                | P    | 20                                  | Mn             | 10                                  |
| 26      | I     | ①                 | 50                                 | 9.1    | 0.17                   | 0.335 | 0.65                                | P    | 15                                  | Mn             | 7                                   |
| 27      | I     | ②                 | 50                                 | 10.0   | 0.17                   | 0.187 | 0.70                                | P    | 17                                  | Mn             | 10                                  |
| 28      | I     | ②                 | 50                                 | 11.0   | 0.17                   | 0.102 | 1.10                                | P    | 450                                 | Mn, Zn, Al     | 250                                 |
| 29      | I     | ③                 | 50                                 | 8.8    | 0.17                   | 0.350 | 0.65                                | P    | 25                                  | Mn             | 15                                  |
| 30      | I     | ④                 | 50                                 | 8.1    | 0.17                   | 0.414 | 0.60                                | P    | 25                                  | Mn, Zn, Al, Ni | 15                                  |
| 31      | II    | ④                 | 50                                 | 8.2    | 0.17                   | 0.385 | 0.60                                | P    | 40                                  | Mn, Zn, Al, Ni | 20                                  |
| 32      | I     | not applied       | 50                                 | 10.5   | 0.17                   | 0.120 | 1.00                                |      |                                     | not applied    |                                     |
| 33      | I     | not applied       | 50                                 | 10.2   | 0.17                   | 0.370 | 0.70                                |      |                                     | not applied    |                                     |
| 34      | I     | not applied       | 50                                 | 10.0   | 0.17                   | 0.350 | 0.70                                |      |                                     | not applied    |                                     |

  

| Article | Configuration of surface treatment |           |               | Manufacturing method               |                            |           |                      |                |               | Performance evaluation result |                                  |  |  |
|---------|------------------------------------|-----------|---------------|------------------------------------|----------------------------|-----------|----------------------|----------------|---------------|-------------------------------|----------------------------------|--|--|
|         |                                    |           |               | Galvanizing condition              |                            |           | coating              |                |               | Performance evaluation result |                                  |  |  |
|         | Coat                               | structure | Surface layer | Total Al concentration in bath (%) | Alloying temperature (°C.) | Treatment | Friction coefficient | $\alpha$ (ton) | $\beta$ (ton) | $\beta/\alpha$                | Chemical conversion treatability |  |  |
| 1       | A                                  | ZnO       |               | 0.13                               | 500                        | RC        | 0.150                | 4.8            | 6.1           | 1.27                          | Good                             |  |  |
| 2       | A                                  | P—Zn      |               | 0.13                               | 510                        | RC        | 0.155                | 4.7            | 6.2           | 1.32                          | Good                             |  |  |
| 3       | A                                  | P—Zn      |               | 0.13                               | 520                        | RC        | 0.150                | 4.7            | 6.2           | 1.32                          | Good                             |  |  |
| 4       | A                                  | P—Zn      |               | 0.13                               | 530                        | RC        | 0.140                | 4.7            | 6.2           | 1.32                          | Good                             |  |  |
| 5       | A                                  | P—Zn      |               | 0.13                               | 550                        | RC        | 0.140                | 4.8            | 6.2           | 1.29                          | Good                             |  |  |

TABLE 3-continued

|    |             |           |      |     |     |       |     |     |      |      |
|----|-------------|-----------|------|-----|-----|-------|-----|-----|------|------|
| 6  | A           | P—Zn      | 0.13 | 560 | RC  | 0.145 | 4.7 | 6.1 | 1.30 | Good |
| 7  | A           | ZnO       | 0.14 | 520 | RC  | 0.150 | 4.7 | 6.2 | 1.32 | Good |
| 8  | A           | P—Zn      | 0.14 | 520 | RC  | 0.140 | 4.7 | 6.2 | 1.32 | Good |
| 9  | A           | P—Zn      | 0.14 | 520 | RC  | 0.140 | 4.7 | 6.2 | 1.32 | Good |
| 10 | A           | P—Zn      | 0.14 | 520 | RC  | 0.145 | 4.7 | 6.2 | 1.32 | Good |
| 11 | A           | P—Zn      | 0.14 | 530 | RC  | 0.150 | 4.7 | 6.2 | 1.32 | Good |
| 12 | A           | P—Zn      | 0.13 | 550 | RC  | 0.145 | 4.7 | 6.2 | 1.32 | Good |
| 13 | A           | P—Zn      | 0.13 | 540 | RC  | 0.135 | 4.7 | 6.0 | 1.28 | Good |
| 14 | A           | P—Zn      | 0.13 | 540 | RC  | 0.145 | 4.6 | 6.1 | 1.33 | Good |
| 15 | A           | P—Zn      | 0.15 | 530 | RC  | 0.150 | 4.7 | 6.2 | 1.32 | Good |
| 16 | A           | P—Zn      | 0.14 | 530 | RC  | 0.145 | 4.7 | 6.2 | 1.32 | Good |
| 17 | A           | P—Zn      | 0.14 | 530 | RC  | 0.145 | 4.7 | 6.2 | 1.32 | Good |
| 18 | A           | P—Zn      | 0.13 | 520 | RC  | 0.140 | 4.7 | 6.2 | 1.32 | Good |
| 19 | A           | P—Zn      | 0.13 | 540 | RC  | 0.150 | 4.7 | 6.2 | 1.32 | Good |
| 20 | A           | P—Zn      | 0.13 | 540 | RC  | 0.130 | 4.7 | 6.2 | 1.32 | Good |
| 21 | A           | ZnO       | 0.13 | 500 | RC  | 0.150 | 4.7 | 6.2 | 1.32 | Good |
| 22 | A           | P—Zn      | 0.13 | 520 | RC  | 0.145 | 4.7 | 6.2 | 1.32 | Good |
| 23 | A           | P—Zn      | 0.13 | 550 | RC  | 0.145 | 4.7 | 6.2 | 1.32 | Good |
| 24 | A           | P—Zn      | 0.13 | 540 | RC  | 0.140 | 4.7 | 6.2 | 1.32 | Good |
| 25 | B           | not exist | 0.13 | 480 | Dip | 0.200 | 4.9 | 5.6 | 1.14 | Good |
| 26 | B           | not exist | 0.13 | 480 | Dip | 0.190 | 4.9 | 5.8 | 1.18 | Good |
| 27 | B           | not exist | 0.13 | 520 | EC  | 0.155 | 4.9 | 5.8 | 1.18 | Good |
| 28 | A           | P—Zn      | 0.14 | 530 | RC  | 0.135 | 4.8 | 6.1 | 1.27 | Fair |
| 29 | B           | not exist | 0.14 | 480 | Dip | 0.165 | 5.0 | 5.8 | 1.16 | Good |
| 30 | A           | P—Zn      | 0.15 | 500 | RC  | 0.195 | 4.6 | 5.5 | 1.20 | Good |
| 31 | A           | P—Zn      | 0.13 | 500 | RC  | 0.180 | 4.6 | 5.5 | 1.20 | Good |
| 32 | not applied |           | 0.13 | 500 |     | 0.155 | 4.5 | 5.4 | 1.20 | Good |
| 33 | not applied |           | 0.13 | 480 |     | 0.200 | 4.2 | 5.0 | 1.19 | Good |
| 34 | not applied |           | 0.13 | 480 |     | 0.140 | 5.0 | 6.4 | 1.28 | Good |

The galvanized steel sheets according to the invention have a low friction coefficient, excellent slidability and satisfactory chemical conversion treatability. As compared with the related art, the galvanized steel sheets according to the invention have an extended range for achieving press forming, defined between the wrinkle generating limit and the fracture generating limit.

On the contrary, coating structures of the lubricating coats of the comparative examples 25, 26, 27 and 29 are of type B. Accordingly, the wrinkle generating limit is high and thus the range for achieving press forming is narrower than that of the steel sheet according to an embodiment of the invention. Meanwhile, comparative examples 28, 30 and 31 that have a coating structure of type A, galvanizing layers of these comparative examples 28, 30 and 31 have small chemical conversion treatability due to a large amount of the coating, or do not satisfy the equation regarding the X-ray diffraction intensity ratio I of the  $\zeta$  phase and the  $\delta_1$  phase in the galvanizing layer according to the invention. Accordingly, the fracture generating limit is low and thus the range for achieving press forming is narrower than that of the steel sheet according to an embodiment of the invention.

### Example 2

Next, Example 2 will be described that differs from Example 1 in the galvanizing process.

#### (1) Test Specimen

The composition of sample steel sheets are shown in Table 1. Cold-rolled steel sheets with 0.7 mm thickness were used.

#### (2) Galvanization Conditions

The test specimen was degreased, washed in acid, and then pre-plated with Ni by electroplating in a Watt bath. The test specimen was then heated to 470°C. in a 4% H<sub>2</sub>—N<sub>2</sub> atmo-

sphere, immersed in a hot dip galvanizing bath of 460°C. for 3 s and then wiped to control the amount. The test specimen was then heated and alloyed under the conditions shown in Table 4, air-cooled to 450°C., subsequently mist-cooled and taken out.

#### (3) Analysis of Galvanizing Layer

The amounts of Zn, Fe, Al and Ni in the galvanizing layer were measured by inductively coupled plasma (ICP atomic emission spectrometry) after the galvanizing layer was dissolved with inhibitor-containing hydrochloric acid to which 0.6% of hexamethylenetetramine manufactured by WAKO Corporation Limited was added. The amounts of Zn, Fe, Al and Ni were summed to obtain the total amount. Other conditions were the same as in Example 1.

#### (4) Conditions for Forming the Coat and Coat Analysis

Conditions for forming the coat and the process of the coat analysis were the same as in Example 1.

#### (5) Performance Evaluation Test

Friction coefficient, wrinkle and fracture generating limits and chemical conversion treatability were similarly evaluated as Example 1.

The performance evaluation results are shown in Table 4. In Table 4, 35 to 50 relate to galvanized steel sheets according to an embodiment of the invention and 51 to 57 relate to galvanized steel sheets according to comparative examples. FIG. 8 shows examples of the present invention and comparative examples in Table 4, with the horizontal axis that represents X-ray diffraction intensity ratio I of the  $\zeta$  phase and the  $\delta_1$  phase regarding the ratio of the  $\zeta$  phase and the  $\delta_1$  phase in the galvanizing layer, and the vertical axis that represents the value obtained by dividing the lower limit wrinkle suppressing force ( $\beta$ ) with which fractures occur by the lower limit wrinkle suppressing force ( $\alpha$ ) which is required for eliminating wrinkles.

TABLE 4

| Article | Steel | Treating solution | Configuration of surface treatment |        |                        |                        |                       |              |                                     |                | Coating layer                       |      |  |  |
|---------|-------|-------------------|------------------------------------|--------|------------------------|------------------------|-----------------------|--------------|-------------------------------------|----------------|-------------------------------------|------|--|--|
|         |       |                   | Galvanizing layer                  |        |                        |                        | Inorganic oxide       |              |                                     | Metallic oxide |                                     |      |  |  |
|         |       |                   | Applied amount (g/m <sup>2</sup> ) | Fe (%) | Al (g/m <sup>2</sup> ) | Ni (g/m <sup>2</sup> ) | Value of equation (1) | Γ phase (μm) | Applied amount (mg/m <sup>2</sup> ) | Type           | Applied amount (mg/m <sup>2</sup> ) | Type |  |  |
| 35      | I     | (1)               | 20                                 | 9.0    | 0.19                   | 0.21                   | 0.250                 | 0.60         | P                                   | 15             | Mn, Zn, Al, Ni                      | 10   |  |  |
| 36      | I     | (1)               | 30                                 | 9.3    | 0.20                   | 0.22                   | 0.210                 | 0.65         | P                                   | 20             | Mn, Zn, Al, Ni                      | 15   |  |  |
| 37      | I     | (1)               | 45                                 | 9.3    | 0.23                   | 0.22                   | 0.195                 | 0.60         | P                                   | 30             | Mn, Zn, Al, Ni                      | 20   |  |  |
| 38      | II    | (1)               | 60                                 | 9.6    | 0.26                   | 0.23                   | 0.174                 | 0.65         | P                                   | 50             | Mn, Zn, Al, Ni                      | 20   |  |  |
| 39      | I     | (2)               | 70                                 | 9.1    | 0.28                   | 0.21                   | 0.310                 | 0.65         | P                                   | 50             | Mn, Zn, Al, Ni                      | 30   |  |  |
| 40      | I     | (2)               | 50                                 | 10.2   | 0.25                   | 0.22                   | 0.117                 | 0.80         | P                                   | 30             | Mn, Zn, Al, Ni                      | 25   |  |  |
| 41      | I     | (2)               | 50                                 | 10.5   | 0.25                   | 0.21                   | 0.065                 | 1.00         | P                                   | 35             | Mn, Zn, Al, Ni                      | 30   |  |  |
| 42      | II    | (2)               | 50                                 | 10.7   | 0.20                   | 0.40                   | 0.080                 | 1.10         | P                                   | 40             | Mn, Zn, Al, Ni                      | 30   |  |  |
| 43      | I     | (3)               | 20                                 | 9.0    | 0.31                   | 0.08                   | 0.210                 | 0.65         | P, B                                | 15             | Mn, Zn, Al, Ce                      | 10   |  |  |
| 44      | I     | (3)               | 30                                 | 9.3    | 0.32                   | 0.09                   | 0.160                 | 0.70         | P, B                                | 25             | Mn, Zn, Al, Ce                      | 15   |  |  |
| 45      | I     | (3)               | 45                                 | 9.2    | 0.35                   | 0.10                   | 0.205                 | 0.60         | P, B                                | 40             | Mn, Zn, Al, Ce                      | 20   |  |  |
| 46      | II    | (3)               | 60                                 | 9.0    | 0.38                   | 0.10                   | 0.201                 | 0.60         | P, B                                | 50             | Mn, Zn, Al, Ce                      | 20   |  |  |
| 47      | I     | (4)               | 30                                 | 10.5   | 0.20                   | 0.22                   | 0.110                 | 0.90         | P                                   | 25             | Mn, Zn, Al, Ni                      | 25   |  |  |
| 48      | I     | (4)               | 45                                 | 9.7    | 0.23                   | 0.21                   | 0.166                 | 0.65         | P                                   | 30             | Mn, Zn, Al, Ni                      | 30   |  |  |
| 49      | I     | (4)               | 60                                 | 10.2   | 0.26                   | 0.21                   | 0.150                 | 0.70         | P                                   | 35             | Mn, Zn, Al, Ni                      | 35   |  |  |
| 50      | II    | (4)               | 70                                 | 9.3    | 0.40                   | 0.08                   | 0.130                 | 0.70         | P                                   | 50             | Mn, Zn, Al, Ni                      | 40   |  |  |
| 51      | I     | (1)               | 50                                 | 9.0    | 0.24                   | 0.20                   | 0.340                 | 0.65         | P                                   | 15             | Mn                                  | 5    |  |  |
| 52      | I     | (2)               | 50                                 | 10.0   | 0.24                   | 0.21                   | 0.170                 | 0.75         | P                                   | 25             | Mn                                  | 10   |  |  |
| 53      | I     | (3)               | 50                                 | 10.8   | 0.36                   | 0.09                   | 0.110                 | 1.00         | P, B                                | 25             | Mn                                  | 15   |  |  |
| 54      | I     | (4)               | 50                                 | 10.1   | 0.24                   | 0.21                   | 0.250                 | 0.70         | P                                   | 20             | Mn                                  | 10   |  |  |
| 55      | I     | (1)               | 50                                 | 11.6   | 0.39                   | 0.10                   | 0.040                 | 1.30         | P                                   | 20             | Mn, Zn, Al, Ni                      | 15   |  |  |
| 56      | I     | (2)               | 50                                 | 11.7   | 0.39                   | 0.11                   | 0.030                 | 1.20         | P                                   | 30             | Mn, Zn, Al, Ni                      | 15   |  |  |
| 57      | I     | (4)               | 50                                 | 11.8   | 0.27                   | 0.22                   | 0.030                 | 1.30         | P                                   | 40             | Mn, Zn, Al, Ni                      | 30   |  |  |

  

| Article | Coat structure | Configuration of surface treatment |      |                  | Manufacturing method            |                                |                            | Performance evaluation result |                      |         |         |     |                                  |  |
|---------|----------------|------------------------------------|------|------------------|---------------------------------|--------------------------------|----------------------------|-------------------------------|----------------------|---------|---------|-----|----------------------------------|--|
|         |                | Galvanizing condition              |      |                  | Coating                         |                                |                            |                               |                      |         |         |     |                                  |  |
|         |                | Coating layer                      | Ni   | Surface layer Zn | pre-plating (g/m <sup>2</sup> ) | Total Al concentration in bath | Alloying temperature (°C.) | condition treatment           | Friction coefficient | α (ton) | β (ton) | β/α | Chemical conversion treatability |  |
| 35      | A              | ZnO                                | 0.30 | 0.18             | 510                             | RC                             | 0.135                      | 4.8                           | 6.2                  | 1.29    | Good    |     |                                  |  |
| 36      | A              | P—Zn                               | 0.30 | 0.18             | 520                             | RC                             | 0.129                      | 4.8                           | 6.3                  | 1.31    | Good    |     |                                  |  |
| 37      | A              | P—Zn                               | 0.30 | 0.18             | 540                             | RC                             | 0.135                      | 4.8                           | 6.4                  | 1.33    | Good    |     |                                  |  |
| 38      | A              | P—Zn                               | 0.30 | 0.18             | 540                             | RC                             | 0.120                      | 4.8                           | 6.4                  | 1.33    | Good    |     |                                  |  |
| 39      | A              | P—Zn                               | 0.30 | 0.18             | 540                             | RC                             | 0.150                      | 4.7                           | 6.2                  | 1.32    | Good    |     |                                  |  |
| 40      | A              | P—Zn                               | 0.30 | 0.19             | 550                             | RC                             | 0.130                      | 4.8                           | 6.4                  | 1.33    | Good    |     |                                  |  |
| 41      | A              | P—Zn                               | 0.30 | 0.19             | 560                             | RC                             | 0.120                      | 4.9                           | 6.2                  | 1.27    | Good    |     |                                  |  |
| 42      | A              | P—Zn                               | 0.50 | 0.19             | 540                             | RC                             | 0.135                      | 4.8                           | 6.1                  | 1.27    | Good    |     |                                  |  |
| 43      | A              | ZnO                                | 0.15 | 0.18             | 500                             | RC                             | 0.132                      | 4.8                           | 6.2                  | 1.29    | Good    |     |                                  |  |
| 44      | A              | P—Zn                               | 0.15 | 0.18             | 510                             | RC                             | 0.127                      | 4.8                           | 6.3                  | 1.31    | Good    |     |                                  |  |
| 45      | A              | P—Zn                               | 0.15 | 0.18             | 530                             | RC                             | 0.120                      | 4.8                           | 6.4                  | 1.33    | Good    |     |                                  |  |
| 46      | A              | P—Zn                               | 0.15 | 0.18             | 530                             | RC                             | 0.115                      | 4.8                           | 6.4                  | 1.33    | Good    |     |                                  |  |
| 47      | A              | P—Zn                               | 0.30 | 0.18             | 530                             | RC                             | 0.125                      | 4.8                           | 6.3                  | 1.31    | Good    |     |                                  |  |
| 48      | A              | P—Zn                               | 0.30 | 0.18             | 540                             | RC                             | 0.120                      | 4.8                           | 6.4                  | 1.33    | Good    |     |                                  |  |
| 49      | A              | P—Zn                               | 0.30 | 0.18             | 540                             | RC                             | 0.140                      | 4.8                           | 6.4                  | 1.33    | Good    |     |                                  |  |
| 50      | A              | P—Zn                               | 0.15 | 0.18             | 540                             | RC                             | 0.140                      | 4.8                           | 6.2                  | 1.29    | Good    |     |                                  |  |
| 51      | B              | not exist                          | 0.30 | 0.18             | 480                             | Dip                            | 0.160                      | 5.0                           | 5.9                  | 1.18    | Good    |     |                                  |  |
| 52      | B              | not exist                          | 0.30 | 0.18             | 500                             | Dip                            | 0.140                      | 5.0                           | 6.0                  | 1.20    | Good    |     |                                  |  |
| 53      | B              | not exist                          | 0.15 | 0.18             | 550                             | EC                             | 0.120                      | 5.0                           | 6.0                  | 1.20    | Good    |     |                                  |  |
| 54      | B              | not exist                          | 0.30 | 0.19             | 500                             | EC                             | 0.150                      | 5.0                           | 6.0                  | 1.20    | Good    |     |                                  |  |
| 55      | A              | P—Zn                               | 0.15 | 0.20             | 550                             | RC                             | 0.110                      | 5.0                           | 5.8                  | 1.16    | Good    |     |                                  |  |
| 56      | A              | P—Zn                               | 0.15 | 0.20             | 550                             | RC                             | 0.110                      | 5.0                           | 5.8                  | 1.16    | Good    |     |                                  |  |
| 57      | A              | P—Zn                               | 0.30 | 0.20             | 550                             | RC                             | 0.100                      | 5.0                           | 5.8                  | 1.16    | Good    |     |                                  |  |

The galvanized steel sheets according to the invention have a low friction coefficient, excellent slidability and satisfactory chemical conversion treatability. As compared with the comparative examples (i.e., the related art), the galvanized steel sheets according to the invention have an extended range for achieving press forming, defined between the wrinkle generating limit and the fracture generating limit. As compared with the galvanized steel sheet according to an embodiment

60 of the invention shown in Table 3 (Example 1), the galvanized steel sheet of Example 2 has an extended range for achieving press forming.

65 In the present invention, both the component having the adhesion-preventing function and the component having the

#### INDUSTRIAL APPLICABILITY

21

rolling-lubricating function are mixed into the entire lubricating coat even in the outermost layer thereof, and in addition, Zn in the lubricating coat is provided even in the outermost layer. A predetermined amount of the  $\zeta$  phase is made to exist on the surface of the galvanizing layer. A synergistic effect generated by the lubricating coat and the galvanizing layer can extend the range for which the galvanized steel sheet can be press formed. As a result, a higher yield can be obtained in the press forming of steel sheets for automobile bodies and the steel sheets can be produced more efficiently than in the related art. In addition, the possibility of the die and punch design can be expanded to produce variously designed press-formed articles, thereby providing automobiles of increased commercial value. Accordingly, the present invention has wide industrial applicability.

BRIEF DESCRIPTION OF REFERENCE  
SYMBOLS

- K1: line representing background intensity having peak 19 corresponding to  $\delta_1$  phase  
 K2: line representing background intensity having peak 20 corresponding to phase  
 L: line representing intensity of  $\delta_1$  (d=0.127 nm) after removal of background intensity in  $\delta_1$  phase  
 M: line representing intensity of  $\zeta$  (d=0.126 nm) after removal of background intensity in phase  
 1: galvanized steel sheet  
 2: steel sheet  
 3: galvanizing layer  
 4: amorphous coating layer (lubricating coat)

The invention claimed is:

1. A galvanized steel sheet comprising:  
 a steel sheet; and  
 a galvanizing layer in an amount of not less than 20 g/m<sup>2</sup> and not more than 100 g/m<sup>2</sup>, the galvanizing layer being provided on a surface of the steel sheet and containing Zn as a main component,  
 wherein the galvanizing layer includes an amorphous coating layer having an inorganic oxoacid salt and metallic oxide on a surface layer of the galvanizing layer;  
 the inorganic oxoacid salt includes oxygen acid salts containing P;

22

the metallic oxide includes:  
 oxides or hydroxides of Zn; and  
 one or more selected from oxides and hydroxides which contain one or more of Al, Mn, Mo, Co, Ni, Ca, V, W, Ti, and Ce;

the galvanizing layer includes a  $\zeta$  phase and a  $\delta_1$  phase; the galvanizing layer includes, by mass, 8 to 13% of Fe; Zn in the metallic oxide exists up to an outermost surface layer of the amorphous layer;

5 10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 9999

22

the metallic oxide includes:  
 oxides or hydroxides of Zn; and  
 one or more selected from oxides and hydroxides which contain one or more of Al, Mn, Mo, Co, Ni, Ca, V, W, Ti, and Ce;

the galvanizing layer includes a  $\zeta$  phase and a  $\delta_1$  phase; the galvanizing layer includes, by mass, 8 to 13% of Fe; Zn in the metallic oxide exists up to an outermost surface layer of the amorphous layer;

5 10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 4

UNITED STATES PATENT AND TRADEMARK OFFICE  
**CERTIFICATE OF CORRECTION**

PATENT NO. : 8,852,753 B2  
APPLICATION NO. : 13/521302  
DATED : October 7, 2014  
INVENTOR(S) : Matsumura Kenichiroh et al.

Page 1 of 1

It is certified that error appears in the above-identified patent and that said Letters Patent is hereby corrected as shown below:

In the Specification

Column 11, line 9, change “amount of the phase” to -- amount of the  $\zeta$  phase --;  
Column 14, line 3, change “ $3 \mu\text{m} \times 3 \mu\text{m}$ ” to --  $3 \mu\text{m} \times 3 \mu\text{m}$  --;  
Column 16, Table 3, for Article 24, under column  $\Gamma$  phase ( $\mu\text{m}$ ), change “0.60” to -- 0.65 --;  
Column 21, line 24, change “corresponding to phase” to -- corresponding to  $\zeta$  phase --; and  
Column 21, line 28, change “intensity in phase” to -- intensity in  $\zeta$  phase --.

Signed and Sealed this  
Twelfth Day of May, 2015



Michelle K. Lee  
Director of the United States Patent and Trademark Office